

Nov. 22, 1966

R. F. SHANNON ET AL

3,286,785

HIGH TEMPERATURE RESISTANT ACOUSTICAL BOARD

Filed May 24, 1965



3,286,785

**HIGH TEMPERATURE RESISTANT  
ACOUSTICAL BOARD**

Richard F. Shannon, Lancaster, and Jerry L. Helser, Hebron, Ohio, assignors to Owens-Corning Fiberglas Corporation, a corporation of Delaware

Filed May 24, 1965, Ser. No. 457,984  
12 Claims. (Cl. 181—33)

The present invention concerns structural, acoustical and thermal insulating boards which are capable of retaining their integrity and dimensional stability at temperatures in excess of 1000° F., and particularly low density siliceous fiber boards possessing an inorganic lamina at one surface and within the voids existing in the fibrous low density structure.

Structural and decorative elements formed from interbonded or intermeshed siliceous fibers, such as glass, mineral wool or asbestos fibers, have achieved extensive use in applications such as ceiling and wall tiles, panels or boards, in which they provide excellent acoustical and thermal insulating properties. Such elements normally comprise an integral, relatively rigid, mass of fibers grouped into a thin panel-like structure having two major opposed and substantially parallel surfaces, a thickness in the order of one-tenth or less of the major dimension of the structure, and possessing a density in the range of 1 to 30 pounds per cubic foot. Due to the non-combustibility of the siliceous fibers, such structures are also valued for their fire resistance.

However, in recent years public concern has shifted to the fire resistance of the total structure as opposed to the combustibility of its individual elements. It was then found that these non-combustible elements contribute to flame spread or building collapse as the result of this loss of integrity at temperatures experienced during a fire. In the first instance, these non-combustible elements are commonly employed to mask or seal off such readily combustible elements as wooden studs, joists, partitions, decking, and the like. At relatively low temperatures, e.g. 500° F., these low density materials perform the desired function in an adequate fashion in both thermally insulating the combustible materials which they conceal and thereby preventing the transfer of temperatures adequate to initiate combustion, and in physically blocking direct flame transfer. However, at higher temperatures, e.g. 1000° F., and despite their own incombustibility, these elements undergo structural failures which permit the transfer of heat or flame to the combustible elements. Such failures result from the sagging, slumping, warping, shrinking, relamination or complete disintegration of the incombustible boards and the ignition of the combustible elements occurs in one of several manners. For example, the sagging, slumping, warping or shrinking of the elements results in their separation from their fastening or suspension means and the formation of a gap or opening between abutting or adjacent boards. Such apertures permit the transfer of heat and/or flame capable of igniting combustible materials located behind the incombustible boards. Alternatively, delamination or disintegration provides apertures for heat or flame transfer through the fibrous boards.

In addition, heat or flame transfer through these siliceous fiber boards may also weaken concealed non-combustible structural elements such as steel beams or girders and concrete decks, to cause a partial or total collapse of the building structure.

As a consequence of this discovery many localities have amended building codes to require prolonged resistance to flame and heat transfer at high temperatures, and particularly in public buildings. Insurance rates have also been adjusted in recognition of this hazard since a build-

ing may be saved if the ignition of combustible structural elements can be avoided.

Accordingly, methods and tests for measuring the resistance of a structure to flame and heat transfer, and the consequent spreading of the fire, have been developed. 5 Typical of such tests and the resultant standards, are the Underwriters Laboratory fire rating tests in which the thermal-acoustical boards are erected in their usual manner of installation, within a furnace chamber approximating the dimensions of a room. Thermocouples are then positioned on the top side of a concrete deck below which is suspended the board to be tested. Flames are then ignited within the chamber and the temperature is progressively elevated, i.e. 1000° F., five minutes after the initiation of the test, 1700° F. at one hour, 1850° F. at 10 2 hours, etc., to simulate the conditions which would be experienced during an actual fire. The test is terminated whenever any of the thermocouples sense temperatures which would be adequate to ignite combustible building 15 elements or to weaken noncombustible elements such as steel beams or concrete decks. This test yields a fire rating based upon the length of endurance of the medium tested under the prescribed conditions. For example, an acoustical board which endured for one hour before permitting the transfer of temperatures adequate to initiate 20 combustion or cause the collapse of noncombustible elements would receive a one hour rating. A failure is experienced whenever any single thermocouple reaches 325° F., above ambient temperature, or when the average 25 temperature of the thermocouples reaches 250° F., above ambient temperature. This test has been described in detail in order to illustrate the improvements made possible by the inventive materials, in terms of the conditions which must be endured.

30 Consequently, the present invention is directed to the provision of low density decorative and structural elements formed from siliceous fibers, which exhibit structural integrity and dimensional stability at temperatures in excess of 1000° F., while retaining the acoustical and thermal insulating properties for which they are valued.

Another object is the provision of methods for the preparation of such low density decorative and structural elements.

40 A further object is the provision of impregnants capable of imparting the prescribed integrity to such decorative and structural elements.

Structural integrity, as used herein, is employed to define the ability to resist the transfer of heat and flames through apertures resulting from the delamination or 45 disintegration of the structure, or through apertures resulting from the separation of the low density boards from their fastenings, suspension systems or from abutting, adjacent boards, upon exposure to temperatures in excess of 1000° F. Consequently, the term "structural integrity" contains an aspect of dimensional stability in respect

50 to resistance to shrinkage, expansion and warping or sagging. It should also be noted that the acoustical properties of the structures include both sound absorption and resistance to sound transmission. The former is provided by the low density, void-filled region which is retained at one major surface of the board, while the latter is improved by virtue of the formation of a dense zone which is substantially impervious to sound at the opposite major surface. At the same time, the insulating values of 55 the boards are enhanced by virtue of the opacifying effect of the dense layer.

60 The above objects and their achievement are described in detail in the following specification and the attached drawings in which:

65 FIGURE 1 is a fragmentary sectional view of a product prepared in accordance with the invention; and,

FIGURE 2 is a schematic representation of an apparatus suitable for the practice of the methods of the invention.

The foregoing objects are achieved by means of the deposition of a thin, continuous inorganic structural phase, or layer, within the voids present within a resin-bonded, low density fibrous medium and immediately adjacent to one of the two major surfaces of the low density fibrous board. The extent of such deposition is limited and controlled in order to prevent the impregnation of the other or opposite major surface, and to thereby retain the desirable thermal and acoustical properties of the low density medium of which the second major surface is composed.

Specifically, an aqueous slurry containing a specific combination of inorganic ingredients formulated to provide the desired structural integrity and dimensional stability, is applied to one surface of the low density fibrous element and then deposited within the voids present in the fibrous medium and adjacent to the point of application. In determining the nature of a layer adequate to provide the prescribed structural integrity, and of the low density zone of the opposite surface adequate to yield the desired acoustical and thermal insulating properties, it has been found that a structural layer having a thickness of 15 mils is adequate, while the acoustical-thermal low density zone or layer must have a thickness of at least 50 mils. However, since the low density boards which are treated in accordance with the invention normally have a thickness of at least 375 mils, the structural layer or impregnated zone normally has a thickness of at least 50 mils while an unimpregnated zone having a thickness of at least 125 mils is preferred.

After depositing and positioning the impregnant to the desired depth, the aqueous component is dispelled by drying to leave a strong rigid structural phase or layer.

*I. Impregnants.*—The inventive impregnants contain both inorganic particulate matter, and a binder phase which is capable of interadhering the inorganic particles both at ambient conditions and during exposure to temperatures in excess of 1000° F. Specifically, the binder phase contains between 5 to 95% by weight of colloidal silica and between 5 to 95% by weight of bentonite, and comprises between 2 to 25% by weight of the total solids present in the impregnant. The impregnant contains between 1 to 20% by weight of colloidal silica and between 1 to 15% by weight of bentonite. It should be noted that references to quantities of colloidal silica relate to the quantities of silica solids, although these compositions are normally employed as dispersions in a liquid carrier medium such as water.

The inorganic particles which are interbonded by the foregoing binder phase include a combination of both materials possessing a melting point below 2000° F., and materials which melt above that temperature. The lower melting materials are the aluminosilicates of the Group I and II metals, sodium, potassium, calcium, magnesium, and barium, and aluminosilicates containing two or more of these metals. The high melting materials comprise certain hydrous aluminum silicates which are subsequently described. This combination is based upon the discovery that the formation of a molten or ceramic phase is highly desirable in the attainment of structural integrity at temperatures experienced during a fire or a fire test.

It is believed that the lower melting materials provide a new or auxiliary adhesive phase upon exposure to temperatures in the range of 1000-2500° F., which serves to interadhere the higher melting particles and to maintain structural integrity. While structural integrity resulting from a "liquid" or molten phase may at first appear contradictory, the nature of this "liquid" must be considered. Specifically, the Group I and/or Group II metals function as fluxes which facilitate the melting of a portion of the ingredients of the impregnant and form an extremely viscous adhesive. For example, molten glass compositions commonly possess viscosities in the range of

10<sup>4</sup> to 10<sup>7</sup> poises and consequently are not highly fluid liquids in the ordinary sense of the word. The value of thermally inert particles interbonded by the described "liquid" adhesive, over thermally inert but structurally weak impregnants is aptly demonstrated by the fire ratings achieved with the inventive impregnants.

The previously described binder phase, i.e. bentonite and colloidal silica, is employed to interbond between 75 to 98% by weight of an admixture of low and high melting materials. In turn, this admixture comprises between 10 to 90% by weight of the higher melting hydrated aluminum silicate particles and between 10 to 90% by weight of the lower melting sodium, potassium, calcium, magnesium and barium aluminosilicates. Consequently, the impregnant composition contains between 7.5 to 90% by weight of both the lower and the higher melting materials.

Thus, the impregnants generally comprise:

|                                       | Percent by weight |
|---------------------------------------|-------------------|
| Colloidal silica (solids)             | 1-20              |
| Bentonite                             | 1-15              |
| Hydrated aluminum silicate            | 7.5-90            |
| Na, K, Ca, Mg and Ba aluminosilicates | 7.5-90            |

Preferably the impregnants contain:

|                           | Percent by weight |
|---------------------------|-------------------|
| Colloidal silica (solids) | 2-6               |
| Bentonite                 | 3-5               |
| Ball clay                 | 30-60             |
| Feldspar                  | 30-60             |

Colloidal silica and silica sols are commercially available compositions and materials of this nature, as well as methods for their preparation, are disclosed by U.S. 2,244,325, 3,083,167, 3,041,140 and 3,128,251.

Bentonite is a commonly known clay mineral composed essentially of montmorillonite and beidellite; it is colloidal hydrated aluminum silicate or sodium montmorillonite.

The hydrated aluminum silicates employed by the invention are ball clays consisting primarily of kaolinite, illite and montmorillonite, with minor quantities of ferric oxide, finely divided silica and titanium dioxide, and trace amounts of lime, magnesia, soda, and potash. More precisely, they contain between 50-75% by weight of SiO<sub>2</sub>, between 15-35% by weight of Al<sub>2</sub>O<sub>3</sub> and between 0.5-10% by weight of Fe<sub>2</sub>O<sub>3</sub> with conventional silica, alumina and iron contents of approximately 57:27:1. Ball clays are distinguished from the more common clays such as kaolin clays, by their lower alumina contents, e.g. 15-35% as opposed to 37-50% for kaolin clays. In addition, between 50-90% of the particles which make up the ball clays employed by the invention have a diameter of 10 microns or less. Furthermore, and as contrasted with the subsequently discussed alkali metal aluminosilicates, the ball clays have a total alkali and alkaline earth metal content of between 0.5-4% by weight. It should be noted that in references made to the quantity of ingredients present in clays or minerals, the total weight of the composition from which the percentages are derived may contain minor quantities of organic materials. Typical of these hydrated aluminum silicates are the Maryland and Tennessee ball clays generally, and such specific materials as Saxon clay, Yankee ball clay, Rex clay, XB ball clay, pyrophyllite, and the like.

The lower melting material is preferably feldspar but one may generally employ the Group I and II metal aluminosilicates of sodium, potassium, calcium, magnesium or barium aluminosilicates, combinations thereof, or aluminosilicates which contain two or more of the specified metal ions, i.e. Na, K, Ca, Ba or Mg. In addition, these metals are present in a quantity of between 6-20% by weight, and preferably 8-15% by weight. Examples of such aluminosilicates include the feldspars such as orthoclase, albite, hydrophane, microcline,

anorthite, anorthoclase, etc.; and such compounds as nepheline, cancrinite, thomsonite, eucryptite, grossularite, alumontite, phillipsite, etc. In addition, the majority of the particles making up these compositions also have diameters of no more than 20 microns.

The examples in the following table provide a number of formulations suitable for use in the present invention, in which the quantities of ingredients are expressed as percentages by weight:

TABLE 1

| Ingredients               | Examples |      |    |      |      |       |    |     |    |
|---------------------------|----------|------|----|------|------|-------|----|-----|----|
|                           | 1        | 2    | 3  | 4    | 5    | 6     | 7  | 8   | 9  |
| Feldspar I                | 47       | 73.3 | 13 | —    | —    | 36.75 | 70 | 76  | —  |
| Feldspar II               | —        | —    | —  | —    | —    | —     | —  | —   | 70 |
| Feldspar III              | —        | —    | —  | 73.5 | —    | —     | —  | —   | —  |
| Nepheline                 | —        | —    | —  | 18.5 | —    | —     | —  | —   | —  |
| Ball clay I               | 47       | 18.3 | 79 | 73.5 | 18.5 | 17    | —  | 17  | —  |
| Ball clay II              | —        | —    | —  | 18.5 | —    | —     | 19 | —   | —  |
| Ball clay III             | —        | —    | —  | —    | 73.5 | 36.75 | —  | —   | —  |
| Colloidal silica (solids) | 2.7      | 5.1  | 3  | 3    | 3    | 3     | 10 | 1.7 | 5  |
| Bentonite                 | 3.3      | 3.3  | 5  | 5    | 5    | 5     | 3  | 3.3 | 8  |

Feldspar I in the above table comprised the following quantities of ingredients expressed in percentages by weight:

|                                      |       |                        |       |
|--------------------------------------|-------|------------------------|-------|
| SiO <sub>2</sub> .....               | 67.53 | CaO.....               | 1.36  |
| Al <sub>2</sub> O <sub>3</sub> ..... | 19.40 | MgO.....               | Trace |
| Fe <sub>2</sub> O <sub>3</sub> ..... | .06   | Na <sub>2</sub> O..... | 6.83  |
| TiO <sub>2</sub> .....               | Trace | K <sub>2</sub> O.....  | 4.58  |
|                                      |       | Organic.....           | .22   |

Its sieve analysis was a residue of 0.3% on a 200 mesh, and 3.2% on a 325 mesh (68.2% of the particles possessed a diameter of 20 microns or less). Feldspars II and III were similar in respect to ingredients and total alkali and alkaline earth metal content, i.e. approximately 12-16% by weight, but feldspar II possessed a higher K<sub>2</sub>O and lower Na<sub>2</sub>O content, while feldspar III contained a higher CaO and MgO content.

Ball clays I and II in the above table contained the following quantities of ingredients and possessed the specified properties:

|                                                                | Ball Clay I | Ball Clay II |
|----------------------------------------------------------------|-------------|--------------|
| SiO <sub>2</sub> .....                                         | 60.19       | 58.66        |
| Al <sub>2</sub> O <sub>3</sub> .....                           | 26.47       | 25.40        |
| Fe <sub>2</sub> O <sub>3</sub> .....                           | 0.89        | 2.29         |
| TiO <sub>2</sub> .....                                         | 1.72        | 1.21         |
| CaO.....                                                       | 0.31        | 0.13         |
| MgO.....                                                       | 0.23        | 0.75         |
| Na <sub>2</sub> O.....                                         | 0.33        | 0.32         |
| K <sub>2</sub> O.....                                          | 0.44        | 2.55         |
| Organic.....                                                   | 9.42        | 8.69         |
| pH.....                                                        | 4.4         | 3.9          |
| Oil absorption (percent).....                                  | 34.5        | —            |
| Residue on 200 mesh (percent).....                             | 0.8         | —            |
| Particles having diameter of 10 microns or less (percent)..... | 81.0        | 93.0         |
| Shrinkage at 2000° F. (percent).....                           | 2.4         | 3.6          |

Ball clay III was similar to ball clay I with the exception that a portion of the aluminum silicate was present as pyrophyllite.

The colloidal silica of the foregoing examples were employed as aqueous dispersions containing between 10-60% by weight of colloidal silica and preferably 40% by weight. However, the quantities recited refer to the amount of silica solids employed.

The impregnants of the above examples were prepared by admixing the ingredients with water to form a slurry. While a slurry containing 20-70%, and preferably 50% by weight of water is preferred in most cases, the ratio must be gauged to yield an impregnant of the viscosity desired for the specific applicator system and substrate employed. For example, in the case of low density fibrous substrates, the viscosity of the impregnant is normally increased by increasing the percentage of solids.

This may be employed to the rate and depth of impregnation. However, the impregnation depth and rate may also be controlled by means independent of the impregnant. For example, vacuum or mechanically pressurized impregnation, e.g. a doctor blade, may be employed to force a highly viscous impregnant to the desired depth within the fibrous substrate. Alternatively, the fibrous substrate may be pre-treated with a wetting agent, e.g. sprayed with a solution of an organosilicone fluid, to fa-

cilitate and control the rate and depth of impregnation by viscous slurries. Similarly, the wetting agent may be incorporated in the impregnant. The siliceous fibers which make up the low density boards treated in accordance with the invention, frequently contain a water repellent which causes the board to resist wetting and penetration by the aqueous slurries which are employed. In such cases, the board should be either pre-treated with a wetting agent, or an agent capable of modifying the surface tension properties of the slurry should be incorporated in the slurry. A wetting agent which has proved highly satisfactory for the above purposes is sodium dioctyl sulfosuccinate having a molecular weight of 444 and available from American Cyanamid under the tradename Aerosol OT.

It should be noted that all of the impregnants of the above examples were applied to siliceous fiber acoustical boards and subjected to a simulated fire test to yield fire ratings in the range of 2-4 hours. These ratings represent a substantial improvement over untreated boards which yield a rating of approximately 15-45 minutes, or boards treated or impregnated with clays, silica, alumina, and the like, which normally provide a one hour rating.

It should also be noted that various other ingredients such as reinforcements, opacifiers, fillers, wetting agents, anti-foaming agents, and the like, may be added to the inventive impregnants. Typical of such additives are, asbestos, asbestine, wollastonite, titania, zircon, zirconia, alumina, carbon black, crystalline silica, calcium carbonate, barium sulfate, magnesium carbonate, ferric sulfate, sodium hexametaphosphate, and the like.

It must also be realized that the inventive combinations of higher and lower melting materials may be simulated by adding fluxing agents to hydrated aluminum silicates having a high melting point, e.g. 2000-3500° F. For example, a fluxing agent such as sodium oxide may be added to a ball clay in a quantity adequate to exert a fluxing effect upon only a portion of the clay, e.g. 8% by weight. Such an expedient also results in a molten or ceramic adhesive phase but is more expensive and difficult to prepare, since minerals which naturally contain a fluxing agent content, e.g. feldspar, are readily available.

**II. Impregnated products.**—As previously mentioned, the products of the invention comprise an acoustical panel, board, or tile formed from siliceous fibers bonded or entangled into a mass having a density in the range of 1 to 30 p.c.f., and possessing two substantially parallel major surfaces, one of which is impregnated with the inventive compositions. The resultant product retains its desirable acoustical and thermal insulating values, while yielding highly improved structural integrity, and resistance to heat or flame transfer when exposed to high tem-

peratures. In order to preserve the acoustical absorption properties of the board, the impregnation of the board throughout its entire thickness, i.e. the filling of all of the voids present in the board, must obviously be avoided. However, satisfactory acoustical properties, and some degree of thermal insulation, are realized when a low density region having a depth of no more than 50 mils is left upon the unimpregnated surface of the board. In turn, an impregnated region having a thickness of no more than 15 mils is adequate to provide structural integrity which permits the board to endure temperatures as high as 2500° F., without failing. It should be realized that in the case of thicker boards, the temperatures which are experienced by the impregnant are lower as the result of the layer of low density thermal insulation which is present at the outside between the impregnant and the heat source.

The acoustical boards comprising glass fibers have an apparent density of from 1 to 30 pounds per cubic foot and are from 250 to 3000 mils thick. These boards impregnated to a depth of at least 15 mils with the treating material.

Preferred embodiments of the invention comprise fibrous glass boards having a density in the range of 8 to 15 p.c.f., a thickness of from 350 to 1500 mils, and an impregnated region having a thickness of about 50 to 750 mils and generally about 50 to 200 mils. Normally, the unimpregnated zone will comprise approximately one-half of the thickness of the board. Examples of such structures comprise a one inch thick board with an impregnated zone or structural layer having a thickness of 50 mils and a  $\frac{1}{8}$  inch thick board having an impregnated zone having a thickness of 500 mils. In the case of boards having a density in the range of 9 to 13 pounds per cubic foot and a thickness of no more than one inch, impregnants constituting between 0.3 to 0.8 pounds per square foot of the impregnated board have proved generally satisfactory. Similarly, a preferred product comprises a board having a density in the range of 9-13 p.c.f., a thickness of between 350 to 1500 mils, and containing between 0.3 and 0.8 pounds of the impregnant present in each square foot of the impregnated board. However, as previously noted, boards having densities of between 1 to 30 p.c.f., and a thickness as great as 3 inches, have been prepared and have yielded the desired properties.

A product prepared in accordance with the invention is depicted by FIGURE 1 which provides a fragmentary, sectional view through a fibrous board prepared in accordance with the invention. As may be seen, one surface 11 of the low density, fibrous board 12 has been impregnated to yield a dense layer 13 which serves as a structural member. As also may be observed, the dense layer 13 also contains the fibers 14 of which the board 12 is composed, and which provide an additional benefit in reinforcing the dense layer 13. In turn, a low density unimpregnated phase 15 is left intact at the opposite surface 16 of the board 12 to provide the desired thermal and acoustical properties.

It should be noted that in the illustrated products the structural value of the dense layer 13 functions primarily after the fibers of the low density unimpregnated phase 15 have been weakened, softened or melted and following pyrolysis of the resin binder. At such time, the dense layer 13 becomes the primary or sole supporting, spanning, or suspending means and may provide the sole source of structural integrity for the board 12.

As previously mentioned, in the use of the inventive impregnants, i.e. containing Group I or II metal alumino-silicate, it is believed that the dense layer 13 does not remain inert upon exposure to temperatures in the range of 1500° F. or higher. Specifically, when inorganic impregnants resistant to temperatures as high as 3000° F. were employed as the dense layer 13, the structures still failed at temperatures far below the melting points of the impregnants. It is believed that such failures were

the result of the absence of an adequate binder phase within the impregnants. In essence, the inert impregnants suffered from thermal erosion or the like, lost integrity, and failed. It was found that the use of the inventive binder phase, i.e. bentonite and colloidal silica, overcame this inadequacy. It was further found that the presence of an ingredient which became molten upon exposure to temperatures in the range of 1500-2500° F., actually improved the integrity of the structure when it was exposed to those temperatures.

The low density fibrous boards employed as the substrate utilized in the above examples and impregnated in the practice of the invention are typified by those disclosed by U.S. 2,790,741; 2,791,289; 2,882,764; 2,984,312; 3,082-143; 3,111,188; 3,118,516; 3,159,235; and similar structures employing glass, mineral wool or asbestos fibers.

In addition, the binder employed to bond the siliceous fibers together into a low density mass, e.g. phenol-formaldehyde or melamine resins, may also contain a fire retardant additive such as clay, asbestos, etc. Alternatively, the fibrous board may be first washed, but not thoroughly impregnated, i.e. without filling the voids throughout the thickness of the board and destroying insulating and acoustical values, with an inorganic material such as a clay slurry, etc. Such measures improve the total fire resistance of the structure although failing to provide adequate structural integrity at high temperatures.

**III. Preparation of the impregnated structures.**—As previously mentioned, the impregnated structures are prepared by depositing a slurry of the inventive impregnant upon one surface of the fibrous board, introducing the impregnant within the voids present upon one surface of the porous board without filling the voids present upon the opposite surface of the board, and drying the impregnant.

A method for fabricating these products is depicted by FIGURE 2 which shows a schematic representation of apparatus suitable for the impregnation of low density siliceous fiber substrates. As shown, fibrous boards 21 are carried by means of a foraminous conveyor belt 22 beneath a trough 23 which dispenses an impregnating slurry 24 upon the upper surface 25 of the boards 21. The deposited impregnant 226 is then passed beneath a metering knife blade 27 which controls the thickness and consequently the quantity of the deposited impregnant 26. The boards 21 are then passed beneath and in contact with a pressure roll 28 which forces the deposited impregnant within the upper surface of the boards 21. To facilitate and control the depth of penetration of the boards 21 by the impregnant, the boards 21 and foraminous conveyor belt 22 may then be passed over a suction box 29 which serves to draw the impregnant within the boards 21 and may implement or replace the effect of the pressure roll 28. Alternatively, or in conjunction with the foregoing process, a sprinkler 30 may deposit a wetting agent such as a silicone fluid upon the upper surface 25 of the boards 21 prior to the deposition of the impregnant. The use of such a wetting agent facilitates the rapidity and extent of the penetration of the boards 21 by the impregnant. The drying of the impregnant may be accomplished by conventional oven treatments. For example, boards having a density of approximately 11.5 p.c.f., a thickness of between 350 to 1000 mils, and containing an impregnant layer weighing approximately 0.8 pounds (aqueous slurry, 50% solids) per square foot of the board, may be oven dried at a temperature of 400° F., in approximately one hour.

Obviously, the primary sources of control for both the rapidity and the degree of impregnation reside in the matching of the viscosity and/or surface tension of the impregnant in relation to the density of the board, the slurry may be merely metered and evenly deposited upon the upper surface of the board, and will immediately

flow to a desired depth within the upper surface of the board, without penetrating to the opposite surface.

In the impregnation of a fibrous glass board having a density of 9-13 p.c.f., it is preferred to employ a slurry having a viscosity of approximately 100-200 centipoises. In such case, the slurry flows entirely within the board to a depth of approximately 125-180 mils within a matter of 1 to 3 seconds.

While the majority of the specification has concerned glass fibers, it must be realized that boards of a comparable density prepared from other siliceous fibers, e.g. mineral wool, asbestos, etc., are equally benefited by the practices of the invention, and yield products which simultaneously provide thermal and acoustical insulating values and prolonged structural integrity at temperatures in excess of 1000° F.

It is obvious that the present invention provides fire resistant, structural integrity imparting impregnants; acoustical and thermal insulating structural elements capable of retaining their integrity at high temperatures; and methods for the preparation of the foregoing structural elements.

The treating materials of this invention can also be used for bonding aggregates such as vermiculite, perlite, glass foam pellets, glass beads and the like to produce products such as high temperature resistant pipe insulation. Likewise these treating compositions can be used for near total impregnation coupled with one or more back-coatings to provide novel effects. The coatings can be used for steel and wood decks to provide improved fire ratings.

It is further apparent that various alterations and substitutions may be made in the compositions, products and methods without departing from the spirit of the invention as defined by the following claims.

We claim:

1. An acoustical and thermal insulating element capable of maintaining structural integrity at temperatures in excess of 1000° F., comprising a plurality of siliceous fibers interbonded into an integral, void-containing mass having a density of between 1 to 30 pounds per cubic foot and shaped in the form of a panel having two substantially parallel major surfaces and a thickness of between 250 and 3000 mils, and deposited within said voids present between said fibers and adjacent to one of said surfaces and to a depth of at least 15 mils, an impregnant comprising between 75 to 98% by weight of aluminum silicate particles consisting essentially of between 10 to 90% by weight of hydrated aluminum silicate containing between 50 to 75% by weight of  $\text{SiO}_2$  and between 15 to 35% by weight of  $\text{Al}_2\text{O}_3$ , and between 10 to 90% by weight of an aluminosilicate of a metal selected from the group consisting of sodium, potassium, calcium, magnesium, barium and combinations of said metals, in which said metal is present in a quantity in excess of 6% by weight, and admixed with and interadhering said aluminum silicate particles between 2 to 25% by weight of a binder phase consisting essentially of between 1 to 20% by weight of colloidal silica and between 1 to 15% by weight of bentonite, the remainder of said panel and the portion of said panel immediately adjacent to the second of said major surfaces to a depth of at least 50 mils being substantially devoid of said impregnant and retaining said density of 1 to 30 pounds per cubic foot.

2. An acoustical and thermal insulating element as claimed by claim 1 in which said siliceous fibers are glass fibers.

3. An acoustical and thermal insulating element as claimed by claim 1 in which said aluminosilicate of a metal is feldspar.

4. An acoustical and thermal insulating element capable of maintaining structural integrity at temperatures in excess of 1000° F., comprising a plurality of glass fibers interbonded into an integral void-containing mass having a density of between 8 to 15 pounds per cubic foot and

shaped in the form of a panel having two substantially parallel major surfaces and a thickness of between 350 to 1500 mils, and deposited within said voids present between said fibers and adjacent to one of said surfaces and to a depth of at least 15 mils, an impregnant comprising between 75 to 98% by weight of aluminum silicate particles and consisting essentially of between 10 to 90% by weight of hydrated aluminum silicate containing between 50 to 75% by weight of  $\text{SiO}_2$  and between 15 to 35% by weight of  $\text{Al}_2\text{O}_3$ , and between 10 to 90% by weight of an aluminosilicate of a metal selected from the group consisting of sodium, potassium, calcium, magnesium, barium and combinations of said metals, in which said metal is present in a quantity in excess of 6% by weight, and admixed with and interadhering said aluminum silicate particles between 2 to 25% by weight of a binder phase consisting essentially of between 1 to 20% by weight of colloidal silica and between 1 to 15% by weight of bentonite, the remainder of said panel and the portion of said panel immediately adjacent to the second of said major surfaces to a depth of at least 50 mils being substantially devoid of said impregnant and retaining said density of 8 to 15 pounds per cubic foot.

5. A method for the preparation of acoustical and thermal insulating elements capable of maintaining structural integrity at temperatures in excess of 1000° F., comprising applying to one major surface of a panel comprising a plurality of siliceous fibers interbonded into an integral void-containing mass having a density of between 1 to 30 pounds per cubic foot and having two substantially parallel major surfaces and a thickness of between 250 to 3000 mils, an aqueous dispersion of an impregnant comprising between 75 to 98% by weight of aluminum silicate particles and consisting essentially of between 10 to 90% by weight of hydrated aluminum silicate containing between 50 to 75% by weight of  $\text{SiO}_2$  and between 15 to 35% by weight of  $\text{Al}_2\text{O}_3$ , and between 10 to 90% by weight of an aluminosilicate of a metal selected from the group consisting of sodium, potassium, calcium, magnesium, barium and combinations of said metals, in which said metal is present in a quantity in excess of 6% by weight, and between 2 to 25% by weight of a binder phase consisting essentially of between 1 to 20% by weight of colloidal silica and between 1 to 15% by weight of bentonite, depositing said dispersion within the voids present between said fibers adjacent to said one major surface and to a depth of at least 15 mils from said one major surface, maintaining the remainder of said panel and the portion of said panel adjacent to the second of said major surfaces to a depth of at least 50 mils from said second major surface substantially devoid of said aqueous slurry, and drying said panel to remove the aqueous phase of said dispersion.

6. A method as claimed by claim 5 in which suction is applied to said second major surface subsequent to the application of said aqueous dispersion to said one major surface.

7. A method as claimed by claim 5 in which said impregnant is displaced from said one major surface to said voids adjacent to said one major surface by applying mechanical pressure to said aqueous dispersion.

8. A method as claimed by claim 5 in which said siliceous fibers are glass fibers.

9. A method as claimed by claim 5 in which said one surface is treated with a wetting agent prior to said applying of said aqueous dispersion.

10. A method as claimed by claim 5 in which said aqueous dispersion also contains a wetting agent.

11. A method for the preparation of acoustical and thermal insulating elements capable of maintaining structural integrity at temperatures in excess of 1000° F., comprising applying to one major surface of a panel comprising a plurality of glass fibers interbonded into an integral void-containing mass having a density of between 8 to 15 pounds per cubic foot and having two substantially parallel

11

major surfaces and a thickness of between 350 to 1500 mils, an aqueous dispersion of an impregnant comprising between 75 to 98% by weight of aluminum silicate particles and consisting essentially of between 10 to 90% by weight of hydrated aluminum silicate containing between 50 and 75% by weight of  $\text{SiO}_2$  and between 15 to 35% by weight of  $\text{Al}_2\text{O}_3$ , and between 10 to 90% by weight of an aluminosilicate of a metal selected from the group consisting of sodium, potassium, calcium, magnesium, barium and combinations of said metals, in which said metal is present in a quantity in excess of 6% by weight, and between 2 to 25% by weight of a binder phase consisting essentially of between 1 to 20% by weight of colloidal silica and between 1 to 15% by weight of bentonite, said fibers adjacent to said one major surface and to a depth of at least 15 mils from said one major surface, maintaining the remainder of said panel and the portion of said panel adjacent to the second of said major surfaces to a depth of at least 50 mils from said second major surface substantially devoid of said aqueous slurry, and drying said panel to remove the aqueous phase of said dispersion.

12. A heat resistant, integrity-imparting impregnant consisting essentially of an aqueous dispersion of between

5  
10

2 to 25% by weight of a binder phase consisting essentially of between 1 to 20% by weight of colloidal silica and between 1 to 15% by weight of bentonite, and between 75 to 98% by weight of aluminum silicate particles consisting essentially of between 10 to 90% by weight of hydrated aluminum silicate containing between 50 to 75% by weight of  $\text{SiO}_2$  and between 15 to 35% by weight of  $\text{Al}_2\text{O}_3$ , and between 10 to 90% by weight of an aluminosilicate of a metal selected from the group consisting of sodium, potassium, calcium, magnesium, barium and combinations of these, in which said metal is present in a quantity in excess of 6% by weight.

12

#### References Cited by the Examiner

##### UNITED STATES PATENTS

|           |        |                     |         |
|-----------|--------|---------------------|---------|
| 3,017,318 | 1/1962 | Labino et al. ----- | 117—126 |
| 3,077,413 | 2/1963 | Campbell -----      | 117—126 |
| 3,141,809 | 7/1964 | DiMaio et al. ----- | 181—33  |

##### FOREIGN PATENTS

|         |         |                |
|---------|---------|----------------|
| 822,261 | 10/1959 | Great Britain. |
|---------|---------|----------------|

RICHARD B. WILKINSON, Primary Examiner.